

# United States Patent Office

2,882,228

Patented Apr. 14, 1959

1

2,882,228

## METAL WORKING LUBRICANTS

Forrest J. Watson and John E. Weigel, Berkeley, and Francis C. Younger, El Cerrito, Calif., assignors to Shell Development Company, New York, N.Y., a corporation of Delaware

No Drawing. Application June 20, 1955  
Serial No. 516,784

6 Claims. (Cl. 252—32.5)

This invention relates to improved lubricating compositions and more particularly to lubricating oil compositions which are stable, non-corrosive, non-staining and possess extreme pressure and anti-wear properties.

Lubricants which are commercially available for use where extreme pressures, high temperatures and high speeds are encountered, as in metal working operations or gear lubrication, are usually unstable, highly corrosive, cause staining and lack desired extreme pressure properties, thereby causing frequent tool or gear failure and contribute to other failures in the machine in which such lubricants are used.

It is an object of the present invention to provide an improved lubricating composition for use under extreme pressure and temperature conditions. Another object is to provide an improved lubricant, which is stable, non-corrosive and non-staining towards metals. A still further object of this invention is to provide an improved metal working and gear lubricant which possesses good extreme pressure properties. Other objects of this invention will become apparent from the description of the invention.

In accordance with the present invention, a superior extreme pressure lubricant is obtained by incorporating into a mineral oil and/or sulfurized mineral oil, minor amounts of two primary additives, one being a partial ester of a polyhydric alcohol and a carboxylic acid and the other being a particular amine salt of a phosphorus acid represented by the general formula:



wherein R is a hydrocarbyl or halohydrocarbyl and preferably a perhalohydrocarbyl radical, in which the carbon chain can range from 1 to 30 and preferably from 1 to 10 carbon atoms; the X's are the same or different divalent atoms of a non-metallic element of group VI-B of the Periodic Table of Elements; of which the elements oxygen and sulfur are preferred; and Y is hydrogen, R as defined, or XH as defined.

The organic phosphonic and phosphinic acids having the above general formula can be prepared by a number of suitable methods such as reported by Arbuzov (J. Gen. Chem. (U.S.S.R.); 898-900, 1934); Coover (Organic Chemical Bulletin, vol. 23, No. 4, 1951); Kosolapoff's "Organic Phosphorus Compounds" (Wiley and Sons);

2

and in U.S. Patents 2,559,752 and 2,614,990. Compounds of this type include halo-organo phosphinic and phosphonic acids such as halo-hydrocarbon phosphinic acids, halo-hydrocarbon phosphonic acids and more specifically the haloalkanephosphinic and haloalkanephosphonic acids.

The amines which can be used to form salts of the above phosphorus acids include highly branched primary aliphatic amines or secondary aliphatic amines of at least 8 carbon atoms. Of the highly branched primary aliphatic amines, the tertiary alkyl primary amines are preferred and they can be prepared by any suitable means such as described in the U.S. Office of the Publication Board Report No. 88843. Other highly branched primary amines can be prepared by converting primary branched chain alcohols as produced by the Oxo process

from branched chain olefins as fully described by P. W. Sherwood in the Oil and Gas Journal, June 9, 1949, page 71, and in the February 1953 issue of Petroleum Processing, to the corresponding nitriles and converting the nitrile to the amine by catalytic hydrogenation. Another method is to convert alcohols to the corresponding halides and to form the amines derived from the halide in the customary manners such as by reacting with ammonia.

It has been found that the tertiary alkyl primary amines, containing, as the tertiary alkyl radical, the radical of polyisobutylene, polypropylene and mixtures thereof are particularly effective for the present purpose and they constitute a preferred class of amines for the practice of the invention. Accordingly, 1,1,3,3-tetramethylbutylamine (from the amination of diisobutylene), 1,1,3,3,5,5-hexamethylhexylamine (from triisobutylene), 1,1,3,3,5,5,7,7 octamethyloctylamine (from tetraisobutylene) and 1,1,3,3,5,5,7,7,9,9-decamethyldecylamine (from pentaisobutylene) are specific preferred amines, which are suitably used individually or as mixtures thereof. In addition to these tertiary alkyl primary amines, primary tertiary alkylmethylamines, such as 2,2,4,4-tetramethyl pentylamine, 2,2,4,4,6,6-hexamethyl heptylamine and the like are suitable.

Other tertiary branched-chain alkyl primary amines which can be used include the C<sub>8</sub> and higher amines of this type mentioned in U.S. Patents 2,160,058, 2,606,923 and 2,611,782, such as tert-tridecylamine



as well as isooheptyldiethylcarbinyl amine, isooctylethylpropylcarbinylamine, and the like. Primary amines of this type are commercially available from Rohm and Haas Company under the trade name of "Primenes," specific products being "Primene 81-R," which is a mixture of primary alkylamines containing from about 12 to 15 carbon atoms and "Primene JM-R," which is a similar tertiary alkylamine mixture containing an average of about 18 to 24 carbon atoms.

The following are the properties of some amines which can be used to form the amine salts for use in lubricating compositions of this invention.

Table I.—Properties

|                               | Tertiary-Octylamine                               | Alkylamine 81<br>A <sub>1</sub>                                                                                    | Alkylamine JM<br>A <sub>3</sub>                                                                                    |
|-------------------------------|---------------------------------------------------|--------------------------------------------------------------------------------------------------------------------|--------------------------------------------------------------------------------------------------------------------|
| Formula.....                  | t-C <sub>12</sub> H <sub>25</sub> NH <sub>2</sub> | Principally t-C <sub>12</sub> H <sub>25</sub> NH <sub>2</sub> to t-C <sub>15</sub> H <sub>31</sub> NH <sub>2</sub> | Principally t-C <sub>12</sub> H <sub>25</sub> NH <sub>2</sub> to t-C <sub>15</sub> H <sub>31</sub> NH <sub>2</sub> |
| Molecular Weight.....         | 128.....                                          | Principally 185-227.....                                                                                           | Principally 269-353.....                                                                                           |
| Average Molecular Weight..... | 131.....                                          | 191.....                                                                                                           | 301.....                                                                                                           |
| Specific Gravity, 25° C.....  | 0.771.....                                        | 0.812.....                                                                                                         | 0.828.....                                                                                                         |
| Refractive Index, 25° C.....  | 1.423.....                                        | 1.447.....                                                                                                         | 1.455.....                                                                                                         |
| Boiling Point (or range)..... | 137-143° C. (760 mm.).....                        | 5-90% at 210-227° C. (760 mm.).....                                                                                | 5-95% at 275-340° C. (760 mm.).....                                                                                |

The secondary amines which can be used to form salts of the phosphorus acids include secondary amines, preferably aliphatic and cycloaliphatic amines, containing from 10 to 36 carbon atoms. Illustrative of such amines are diethylamine, dihexylamine, di(2-ethylhexyl) amine, di-octylamine, didecylamine, didodecylamine, ditetradecylamine, dihexadecylamine, dioctadecylamine, dibromo-di-octadecylamine, isopropyloleylamine, diricinoleylamine, butyricinoleylamine, butyl-2-ethylhexylamine, dilaurylamine, methyloleylamine, ethyloctylamine, isoamylhexylamine, dicyclohexylamine, dicyclopentylamine, cyclohexyloctylamine, cyclohexylbenzylamine, benzyloctylamine, benzyl-2-ethylhexylamine, allyloctylamine, dodecyl-2-ethylhexylamine, (1-isobutyl-3-methylbutyl)-3,3,5-methylcyclohexylamine, di(1-isobutyl-3-methylbutyl) amine; N-n-dodecylidihylenetriamine, N-n-tetradecylidihylenetriamine, octylethylene diamine, N-2-ethylhexyl N-hexadecyl triethylene tetramine, heptyl trimethylene diamine, N-tetradecyl tripropylene tetramine, N,N'-diallyl trimethylene diamine, 3-hexyl-morpholine, and the like.

The phosphorus acids used to form the partial or full amine salts include such compounds as haloalkanephosphinic acids and haloalkanephosphonic acids such as trichloromethanephosphinic acid, trichloromethanephosphonic acid, 1,1-dibromoethanephosphinic acid, 3,3,5-trichlorocyclohexanephosphinic acid, 1,1-dichlorohexadecanephosphinic acid, 1,1-dichlorohexadecanephosphinic acid; trichloromethanephosphonic acid, 1,1-dichloroethanephosphonic acid, 2,2,2-trichloroethanephosphonic acid, tribromomethanephosphonic acid, dichloromonobromomethanephosphonic acid, 1,1-dibromobutanephosphonic acid, 1,1-dichlorophenylethanephosphonic acid, 3,3,5-trichlorocyclohexanephosphonic acid, 3,5-dichlorocyclohexanephosphonic acid, 1,1-dichloropropaneephosphonic acid, 3,3,3-tribromopropaneephosphonic acid, 1,1-dichloroethanephosphonic acid, 1,1-dichlorobutanephosphonic acid, dichlorophenyl benzenephosphonic acid, 1,1-dichloro-2-monobromobutanephosphonic acid, 1,1-dichlorooctaneephosphonic acid, trichloromethanephosphonic acid, 1,1-dibromobutanethiophosphonic acid, 3,3,5-trichlorocyclohexanethiophosphonic acid, 1,2-dichloroethanethiophosphonic acid, trichloromethaneselenophosphonic acid, and the like.

The phosphorus acid salts can be represented by the general formulas:



(II) 50 or equivalently



(III) 55



(IV)

wherein R and X are the same as in Formula I; R<sub>1</sub> can be hydrogen or R as defined, and A is a long-chain highly branched aliphatic primary amine or aliphatic secondary amine, preferably having at least 8 carbon atoms and higher such as up to 30 carbon atoms in the molecule.

The amine salts of the acidic phosphono compounds and mixtures thereof as described can be prepared by interacting selected amines with polyhalo-organo phosphorus compounds as described above, as in a suitable solvent or in the presence of water and under suitable conditions such as mixing at room temperature, stirring or

heating. Salts produced in the foregoing or equivalent manner can be purified by recrystallization from suitable solvents or other means which will be apparent to those skilled in the art. For example, trichloromethanephosphinic acid was reacted at a temperature of around 50° C. with a mixture of t-C<sub>18</sub>H<sub>37</sub>NH<sub>2</sub> to t-C<sub>24</sub>H<sub>49</sub>·NH<sub>2</sub> (A<sub>3</sub>) in an amount sufficient to neutralize the total acidity of the acid, namely, one mole of the acid for two moles of the amine. The product is represented by the formula



or equivalently



This salt was completely soluble in mineral oil and possessed excellent extreme pressure properties. Using two moles of t-C<sub>12</sub>H<sub>25</sub>NH<sub>2</sub> to t-C<sub>15</sub>H<sub>35</sub>NH<sub>2</sub> (A<sub>1</sub>) in forming the above type of salt, the final product had the formula



or equivalently



Another excellent extreme pressure additive having good oil solubility was prepared in the manner described above using only half the stoichiometric amount of amine (A<sub>3</sub>) required to neutralize the total acidity of trichloromethanephosphonic acid. The product formed had the formula



(II) 50 or equivalently



The partial neutral primary highly-branched-chain amine salts which are specifically preferred include: t-C<sub>12</sub>H<sub>25</sub>NH<sub>2</sub>, t-C<sub>12</sub>H<sub>25</sub>NH<sub>2</sub> to t-C<sub>15</sub>H<sub>31</sub>NH<sub>2</sub>, t-C<sub>18</sub>H<sub>37</sub>NH<sub>2</sub> to C<sub>24</sub>H<sub>49</sub>NH<sub>2</sub>, dimethyl neopentylcarbinyl amine, tert. 65 tridecylamine salts of trichloromethanephosphonic acid, 1,1-dichloroethanephosphonic acid, 1,1-dibromobutaneephosphonic acid, trichlorobenzenephosphonic acid, tribromomethanephosphonic acid, trifluoromethanephosphonic acid, tribromomethanephosphonic acid, trichloromethanephosphonic acid, chlorobenzene trichloromethanephosphinic, 1,1-dichloroethanethiophosphonic acid, trichlorobenzenephosphonic acid, trichloromethanephosphinic acid, dibromoethanephosphonic acid, and mixtures thereof.

The secondary amine salts which are specifically preferred include: di-2-ethylhexylamine, di-1-isobutyl-3-methylbutylamine, didecylamine, dioctadecylamine, isopropyloleylamine, butyl-2-ethylhexylamine, dicyclohexylamine, 1,1-dichloroethanephosphonic acid, 1,1-dibromobutaneephosphonic acid, trichlorobenzenephosphonic acid,

tribromomethanephosphonic acid, trifluoromethanephosphonic acid, tribromomethanephosphonic acid, trichloromethane-dithiophosphonic acid, chlorobenzene trichloromethanephosphinic, 1,1-dichloroethanethiophosphonic acid, trichlorobenzenephosphonic acid, trichloromethanephosphinic acid, dibromoethanephosphinic acid, and mixtures thereof.

Although the primary and secondary amine salts are excellent for use in compositions of this invention, when the secondary amine salts are used, a solubilizer is generally necessary. Solubilizers for this purpose, which do not interfere with the extreme pressure activity of the salts, are oil-soluble aliphatic alcohols and/or thiols, which can be saturated or unsaturated, straight or branched-chain of at least 6 carbon atoms in the molecule. Branched-chain alkanols can be produced by the Oxo process fully described by P. W. Sherwood in the Oil and Gas Journal, June 9, 1949, page 71, and in the February 1953 issue of Petroleum Processing as well as in U.S. Patents 2,571,160 and 2,637,698. Other types of alcohols, such as the straight or branched-chain fatty alcohols, can be used as well as their thiol analogues. Examples of suitable alcohols are: hexyl, heptyl, octyl, nonyl, decyl, dodecyl, tridecyl, tetradecyl, octadecyl, benzyl, cyclohexyl, dimethyl cyclohexyl, 3,3,5-trimethylcyclohexyl, oleyl alcohols, sperm oil alcohol, wool grease alcohol, Oxo C<sub>8</sub>-C<sub>18</sub> alcohols (manufactured by Enjay Company and produced from olefins, carbon monoxide and hydrogen by the Oxo process), Archer-Daniels-Midland "Adols" which are higher fatty alcohols. The thiol analogues of these alcohols, such as described in U.S. Patent 2,638,448, and including iso-octanethiol, decanethiol, octadecanethiol, tertiary tetradecanethiol, tertiary hexadecanethiol and the like or mixtures of said alcohols and/or thiols can be used with the phosphorus compounds in accordance with this invention.

The other primary additives, which produce a synergistic effect when used in combination with the phosphorus compounds, are partial esters of polyhydric alcohols and organic carboxylic acids.

In general, there are utilized partial esters of fatty acids of from about 8 to 32 carbon atoms and wherein the ratio of esterified to unesterified alcoholic groups is from about 1:5 to about 5:1, with those having a ratio of from about 1:2 to 2:1 being preferred, and particularly partial esters of C<sub>10</sub>-C<sub>20</sub> fatty acids and aliphatic polyhydric alcohols.

One group of useful esters comprises those derived from simple water-soluble alkanepolyols of from 2 to 6 carbon atoms such as ethylene glycol, propylene glycol, glycerol, erythritol, pentaerythritol, sorbitol, mannitol, dulcitol and the like. Another group of useful partial esters are those which are esters of water-soluble partially dehydrated (etherified) polyhydric alcohols, including mixed ether-alcohols of different polyhydric alcohols. Partial dehydration converts the simpler ones to linear ether-alcohols and some of the higher ones to an inner ether-alcohol. Thus, for example, ethylene glycol gives rise to diethylene glycol, triethylene glycol, etc., and mannitol, sorbitol and the like give rise to hexitans, such as mannitan and sorbitan. The hexitans can be etherified with alkylene oxides such as ethylene oxide or glycols to give mixed ether-alcohol. Still another group of partial esters suitable for the practice of the invention are the partial esters of water-soluble aldose and ketose carbohydrates generally referred to as the sugar esters.

The acids which can be used to make the partial esters from any of the above alcohols include aliphatic carboxylic acids; cyclic organic carboxylic acids; aromatic carboxylic acids; sulfonic acids and the like. The aliphatic carboxylic acids include the mono- and polycarboxylic acids of from 8 to 32, and preferably from 10 to 20, carbon atoms and include saturated and unsaturated fatty acids of from about 10 to 20 carbon

atoms such as lauric, stearic, oleic and linoleic acids, as well as aliphatic polycarboxylic acids such as alkenyl succinic acid, alkyl adipic acid and the like. The cyclic carboxylic acids include naphthenic acids, such as cyclohexane carboxylic acid, alkylcyclohexane carboxylic acids, alkylcyclopentane carboxylic acid, abietic acid and the like. The aromatic acids include the substituted aromatic carboxylic acids such as benzoic, salicylic, phthalic, anthranilic acids, the alkylated salicylic and anthranilic acids in which the alkyl radical is from 3 to 20 carbon atoms being preferred ones.

Specific esters derived from simple alkanepolyols include glycerol monooleate, glycerol monostearate, glycerol monoricinoleate, pentaerythritol monocaprylate, pentaerythritol mono- and dilaurate, pentaerythritol mono- and dioleate, pentaerythritol mono- and distearate, mono-, di-, and triethylene glycol monooleate, propylene glycol monoricinoleate, monoethylene glycol monooleate, triethylene glycol monostearate, sorbitol monolaurate, mannitol monooleate, mannitol dioleate, sorbitol dioleate, etc.

Esters derived from ether-alcohols as described may be prepared by the method described in U.S. Patent 2,322,820. Examples of such esters which must contain at least one and preferably more than one free hydroxyl group are sorbitan mono- and dioleate, sorbitan mono- and dilaurate, mannitan mono- and distearate, mannitan mono- and dioleate, sorbitan mono- and dipalmitate, sorbitan sesquioleate, sorbitan mononaphthenate, mannitan monolaurate, etc.

Esters derived from the sugar alcohols include glucose monooleate, glucose monoricinoleate, sorbose monostearate, fructose monooleate and the like.

If desired, minor amounts of secondary additives can be used in conjunction with the two primary additives in compositions of this invention. Among such additives are the sulfurized and/or sulfohalogenated fatty materials such as animal, vegetable and marine fats and oils and derivatives thereof. Materials of this type can be prepared by the methods described in U.S. Patents 2,322,859, 2,454,034, 2,459,717, 2,467,137, 2,614,078, 2,644,825 and 2,701,237. Among such materials are sulfurized or sulfo-chlorinated fats fatty oils of the animal, vegetable and marine type and derivatives thereof, such as sulfurized or sulfo-chlorinated tallow, lard, lanolin, jojoba oil, rapeseed oil, sperm oil, fatty acids of these fats and oils as well as their esters such as C<sub>14</sub> to C<sub>20</sub> saturated and unsaturated fatty acids, e.g., myristic, stearic, oleic acids, polymerized fatty acids such as polymerized linoleic acid or "Empol 1022" which is a polymerized fatty acid made by Emery Industries; or esters such as cetyl stearate, cetyl oleate and mixtures thereof; halogenated fats, oils, waxes such as chlorinated paraffin wax, chlorinated tallow, etc., of these materials preferred are the sulfurized sperm oil, lanolin, rapeseed oils, oleic acid chlorinated paraffin wax and cetyl oleate as well as mixtures thereof.

In addition, various oil-soluble anti-oxidants, e.g., alkyl phenols; corrosion inhibitors, e.g., mercaptobenzothiazole and salts thereof, diisopropyl ammonium nitrite, C<sub>8</sub>-C<sub>11</sub> fatty acids; anti-foaming agents, e.g., silicone polymers, organic phosphates, aliphatic alcohols and the like, can be used.

Base oils to which agents of this invention are added may be selected from a variety of natural oils such as paraffinic, naphthenic and mixed base mineral oils having a viscosity range such as from 50 SUS at 100° F., up to 250 SUS at 210° F. In addition, synthetic oils may be used such as polymerized olefins, alkylated aromatics; polyalkyl silicone polymers, e.g., liquid dimethyl silicone polymer, other silicone polymers; H<sub>2</sub>S-adducts of unsaturated ethers and thioethers, e.g., H<sub>2</sub>S adduct of diallyl ether; esters, e.g., di(2-ethylhexyl) sebacate. Mixtures of natural and synthetic oils can be used.

The following is the general formula for compositions of this invention:

| Components                                                                                 | Amounts, Percent Wt. |           |
|--------------------------------------------------------------------------------------------|----------------------|-----------|
|                                                                                            | General              | Preferred |
| <b>Primary Additives:</b>                                                                  |                      |           |
| Amine salt of phosphonic or phosphinic acid                                                | 0.1-10               | 1-5       |
| Partial ester of polyhydric alcohol and organic carboxylic acid or organic sulfurized acid | 0.1-10               | 1-5       |
| <b>Secondary Additives:</b>                                                                |                      |           |
| Alcohol solubilizers                                                                       | 0-5                  | 1-4       |
| Sulfurized fatty material                                                                  | 0-10                 | 1-5       |
| Anti-oxidant, corrosion inhibitor, anti-staining agent                                     | 0-1                  | 0.1-1     |
| <b>Base:</b>                                                                               |                      |           |
| Lubricating oil and/or sulfurized lubricating oil                                          | Balance              | Balance   |

Specific examples of compositions of this invention are:

**Composition A:**

0.5% sulfurized oleic acid  
1.0% glycerol monooleate  
0.75% trichloromethanephosphonic acid  
1.40% Alkylamine 81 (see Table I)  
Bal. SAE 90 mineral oil

**Composition B:**

0.5% sulfurized oleic acid  
1.0% sorbitan dioleate  
0.75% trichloromethanephosphonic acid  
1.40% Alkylamine 81 (see Table I)  
Bal. SAE 90 mineral oil

**Composition C:**

0.5% polymerized fatty acid (Empol 1022)  
0.5% glycerol monooleate  
0.75% trichloromethanephosphonic acid  
1.40% Alkylamine 81 (see Table I)  
1.75% chlorinated paraffin wax  
Bal. SAE 90 mineral oil

**Composition D:**

0.5% polymerized fatty acid (Empol 1022)  
0.5% sorbitan dioleate  
0.75% trichloromethanephosphonic acid  
1.40% Alkylamine 81 (see Table I)  
1.75% chlorinated paraffin wax  
Bal. SAE 90 mineral oil

**Composition E:**

0.2% glycerol monooleate  
0.75% trichloromethanephosphonic acid  
2.6% Alkylamine JM (see Table I)  
1.75% chlorinated paraffin wax  
Bal. SAE 90 mineral oil

**Composition F:**

1.0% glycerol monooleate  
0.75% trichloromethanephosphonic acid  
1.40% Alkylamine 81 (see Table I)  
Bal. SAE 70 mineral oil

**Composition G:**

1.0% sulfurized sperm oil  
1.0% glycerol monooleate  
0.75% trichloromethanephosphonic acid  
0.70% Alkylamine 81 (see Table I)  
0.2% 2-mercaptopbenzothiazole  
Bal. sulfurized pale oil (80 SUS at 210° F.)

**Composition H:**

1.0% glycerol monooleate  
0.75% trichloromethanephosphonic acid  
0.70% Alkylamine 81 (see Table I)  
0.2% 2-mercaptopbenzothiazole  
Bal. sulfurized pale oil (80 SUS at 210° F.)

The superiority of compositions of this invention as extreme pressure and corrosion resistant lubricants is evidenced from the data presented in Table II. The extreme pressure properties of the compositions tested in Table II were determined in the four-ball extreme pressure tester

described in "Engineering," vol. 136, July 13, 1933, and in a hypoid gear testing machine operated at 4,000 r.p.m. pinion speeds at a maximum reversed load and the horsepower developed before failure occurred was noted. The corrosion resistant properties of the compositions were determined by the L-13 test described in the CRC Handbook.

Table II

| 10 | Compositions | Four-Ball Test: Initial Seizure Load (Kg.) | L-13 Corrosion Test | Hypoid Gear Test (H.P.) |      |
|----|--------------|--------------------------------------------|---------------------|-------------------------|------|
|    |              |                                            |                     | 141-158                 | 140+ |
| A  |              | 141-158                                    | Passed              | 140+                    |      |
| B  |              | 126-141                                    | do                  | 140+                    |      |
| C  |              | 141-158                                    | do                  | 140+                    |      |
| D  |              | 126-141                                    | do                  | 112+                    |      |
| E  |              | 126-141                                    | do                  | 140+                    |      |
| F  |              | 126-141                                    | do                  | 140+                    |      |
| G  |              | 178-200                                    | do                  | 140+                    |      |
| H  |              | 178-200                                    | do                  | 140+                    |      |
| 1* |              | 79-89                                      | Failed              | Failed immediately      |      |
| 2  |              | 79-89                                      | do                  | 28                      |      |
| 3  |              | 141-158                                    | do                  | 28                      |      |
| 4  |              | 141-158                                    | do                  | Failed immediately      |      |
|    |              | 79-89                                      | do                  |                         |      |

\*1=Mineral oil (SAE 90)+1% glycerol monooleate.

2=Mineral oil (SAE 90)+1% di-2-ethylhexylamine salt of trichloromethane phosphonic acid.

3=Composition H but from which the glycerol monooleate was omitted.

4=Mineral oil (SAE 90).

Compositions G and H were used in a thread cutting machine and excellent threading of mild steel at speeds of over 1,025 r.p.m. was achieved, while with compositions 1 to 4 threading was poor at speeds of less than 400 r.p.m.

Similar results to those for compositions A to H in the above tests can be achieved by substitution for the trichloromethanephosphonic acid of other acids such as trichlorobenzenephosphonic acid, butyl trichloromethanephosphonic acid, trichloromethanephosphonic acid; and for the Alkylamine 81 or JM of such amines as tertiary octylamine, di-2-ethylhexylamine, dicyclohexylamine; and for the glycerol monooleate or sorbitan dioleate such esters as pentaerythritol monooleate, sorbitol monooleate, mannan monolaurate, glucose monooleate and sorbose monostearate.

Under certain conditions of lubrication, the addition of polyhydric alcohols, such as alkyl glycols, erythritol, glycerin, hexitols and the like, is most advantageous. This is particularly applicable where the lubricating compositions are used under extremely high temperatures and heavy load conditions.

The additive combination of this invention also can be used to improve turbine oils, process oils, industrial oils, hydraulic fluids and heat transfer fluids.

We claim as our invention:

1. A lubricating oil composition comprising a major amount of a mineral lubricating oil containing from about 0.1% to about 10% each of a long chain highly branched primary tertiary aliphatic amine of at least 8 carbon atoms salt of a chloromethanephosphonic acid, and a partial ester of a polyhydric alcohol having from 2 to 6 carbon atoms and a  $C_{10}-C_{20}$  fatty acid.

2. A lubricating oil composition comprising a major amount of a mineral lubricating oil containing from about 0.1% to about 10% each of a long chain highly branched primary tertiary aliphatic amine of at least 8 carbon atoms salt of trichloromethanephosphonic acid and a partial ester of a polyhydric alcohol having from 2 to 6 carbon atoms and a  $C_{10}-C_{20}$  fatty acid.

3. A lubricating oil composition comprising a major amount of a mineral lubricating oil containing from about 0.1% to about 10% each of a long chain highly branched primary tertiary aliphatic amine of at least 8 carbon atoms salt of trichloromethanephosphonic acid and glycerol monooleate.

4. A lubricating oil composition comprising a major amount of a mineral lubricating oil containing from about 0.1% to about 10% each of a long chain highly

branched primary tertiary aliphatic amine of at least 8 carbon atoms salt of trichloromethanephosphonic acid and sorbitan dioleate.

5. A lubricating oil composition comprising a major amount of a mineral lubricating oil containing from about 0.1% to about 10% each of  $t\text{-C}_{12}\text{H}_{25}\text{NH}_2$  to  $t\text{-C}_{15}\text{H}_{31}\text{NH}_2$  salt of trichloromethanephosphonic acid, glycerol monooleate and sulfurized sperm oil.

6. A lubricating oil composition comprising a major amount of a mineral oil containing from about 0.1% to 10 about 10% each of a long chain highly branched tertiary aliphatic amine of at least 8 carbon atoms salt of a

chloromethanephosphonic acid, a partial ester of a polyhydric alcohol having from 2 to 6 carbon atoms and a  $\text{C}_{10}\text{-C}_{20}$  fatty acid and sulfurized sperm oil.

|                       |                                             |
|-----------------------|---------------------------------------------|
| 5                     | References Cited in the file of this patent |
| UNITED STATES PATENTS |                                             |
|                       | 1,463,092 Pelly ----- July 24, 1923         |
|                       | 2,249,800 Weber ----- July 22, 1941         |
|                       | 2,479,424 Sproule ----- Aug. 16, 1949       |
|                       | 2,515,115 Davis ----- July 11, 1950         |
|                       | 2,683,691 Thorpe ----- July 13, 1954        |